

Patented May 7, 1929.

1,711,940

# UNITED STATES PATENT OFFICE.

HARRY LE B. GRAY, OF ROCHESTER, NEW YORK, ASSIGNOR TO EASTMAN KODAK COMPANY, OF ROCHESTER, NEW YORK, A CORPORATION OF NEW YORK.

## PROCESS OF MAKING CELLULOSE ESTERS OF HIGH UNIFORMITY.

No Drawing.

Application filed August 25, 1927. Serial No. 215,518.

This invention relates to processes of making cellulose esters of high uniformity. One object of the invention is to mix the cellulosic material and acylating liquid so thoroughly that uniform esters are ultimately produced. Another object is to impregnate the cellulose with the liquid, prior to esterification, very uniformly, even if the proportion of liquid relative to the cellulose be small. Other objects will hereinafter appear.

In the manufacture of cellulose esters of organic acids it is highly desirable to have the acylation uniform throughout the fibers in order to get a uniformly soluble product. For example, in making cellulose acetate it is desirable to get uniform acetylation in order to prevent the presence of particles in the product which are insoluble or partially insoluble in the customary solvents. Such particles impair the transparency of films, for instance.

It has been customary to mix the cellulose in an excess of the acylating liquid under at least atmospheric pressure. Often the excess is allowed to remain during the esterification. Where only a relatively small proportion of such liquid is to remain for the reaction, the excess is pressed out and removed. There is a tendency for non-uniform mixing under these conditions. Each fiber of cellulose is not fully wetted with the organic liquid and a non-uniform product results.

I have found that air trapped among the fibers or clinging to the latter in the form of small bubbles is a cause of the trouble, and that the latter can be avoided or greatly lessened by putting the cellulose under a vacuum, and impregnating it with the organic acylating liquid while it is under such vacuum. A cellulose ester of great uniformity is obtained from the subsequent acylation at normal pressure.

My invention is applicable to any of the cellulosic fibers useful in making cellulose esters. Since cellulose acetate is at present of major importance, I shall describe, by way of example, the use of acylating liquids in carrying out my process, but it will be understood that my invention is applicable to any similar organic acylating liquids.

The degree of vacuum employed can be varied considerably because some kinds of cellulose are less troublesome than others.

The greater the tendency to retain air, the

higher the vacuum employed. A fairly strong vacuum of 14 to 40 millimeters of mercury gives satisfactory results in nearly all cases.

In applying my invention to the "dope" method of making cellulose acetate, for illustration, 100 parts by weight of clean cotton are placed under a vacuum of 16 mm. in any suitable known vacuum apparatus, the inner walls of which are resistant to the acylating bath. While the vacuum is maintained, there is run into the cotton and thoroughly mixed with it an acylating bath containing 500 parts by weight of glacial acetic acid, 300 parts of acetic anhydrid, and 70 parts of the catalyst, such as 2 parts of magnesium perchlorate trihydrate, or the usual quantities of sulfuric acid, or zinc chlorid. The vacuum is kept up until air bubbles substantially cease to rise from the mixture. At 75 room temperature, this ordinarily does not take over an hour. During this time, instead of a continuous vacuum, the latter may be repeatedly raised and lowered or even broken entirely and then renewed. The vacuum is 80 finally stopped and the esterifying reaction then conducted at substantially atmospheric pressure and under the usual or normal conditions.

My present invention is especially useful 85 for mixing the ingredients in the process disclosed in the application of the present inventor and Cyril J. Staud, Serial No. 196,999, filed June 6th, 1927, for "process of making chloroform-soluble cellulose acetate." 90 In that process the proportion of acylating liquid to the cellulosic solids is very small and the cellulose acetate does not dissolve. Uniformity of impregnation of the cellulose with the acetic anhydrid is especially important to insure that all parts of the fibers shall be converted into chloroform-soluble cellulose acetate without leaving insoluble portions. My present vacuum treatment 95 greatly facilitates the obtaining of this uniformity. For example, 100 parts by weight of filter cotton (a highly purified dewaxed cotton) are placed in a vacuum chamber, the walls of which are acid resistant. A vacuum corresponding to between 14 to 40 105 millimeters of mercury, say 16 mm., is created in the chamber. While the vacuum is kept up, 220 parts by weight of acetic anhydrid (94% strength), containing 0.12 parts by weight of sulfuric acid (98% 110

strength), and 0.12 parts of phosphoric acid (85% strength), is run into the cotton and preferably mixed or agitated with it. A vacuum is maintained for about an hour at 5 room temperature. The vacuum during this period may be increased and decreased or even broken entirely and repeated, in order to facilitate the impregnation. After the latter is complete, the vacuum is released 10 and the acetylation is carried out at atmospheric pressure, as in said application, Serial No. 196,999.

It will be seen that in these examples the cellulose fibers are mixed uniformly with 15 just the right amount of liquid for the subsequent reaction. The liquid, containing from 2 to 5 times as much acetic anhydrid as cellulose, remains in admixture with the cellulose during the subsequent reaction. 20 No excess of liquid is required, and consequently the pressing out and handling of an excess and the deterioration of such excess are avoided.

Having thus described my invention, 25 what I claim as new and desire to secure by Letters Patent is:

1. In the process of making cellulose esters of organic acids the steps of subjecting a mixture of acylating liquid and the cellulose material to be esterified to a vacuum 30 until entrapped air is removed, and thereafter breaking the vacuum and conducting the reaction between said liquid and material.

35 2. In the process of making cellulose esters of organic acids the steps of subjecting the cellulose fibers to be esterified to a vacuum, mingling with said fibers, while a vac-

uum is maintained, the quantity of acylating liquid which is to be present during the 40 reaction, breaking said vacuum when air bubbles have been substantially removed from the mixture, and thereafter conducting the esterifying reaction.

3. In the process of making cellulose acetate the steps of subjecting a reaction mixture of cellulosic fibers and acetylating liquid containing acetic anhydrid and a catalyst to a vacuum to remove entrapped air, 45 breaking said vacuum and then conducting 50 the acetylation reaction.

4. In the process of making cellulose acetate, the steps of subjecting the cellulosic fibers to be acetylated to a vacuum, mingling with said fibers, while a vacuum is 55 maintained, the quantity of acetylating liquid, including acetic anhydrid, which is to be present during the acetylation, breaking the vacuum when air bubbles substantially cease to evolve from the mixture and there- 60 after conducting the acetylation reaction.

5. In the process of making cellulose acetate, subjecting 100 parts by weight of cellulosic fibers to a vacuum corresponding to between 14 and 40 millimeters of mercury, 65 mixing acetylating liquid containing 200 to 500 parts of acetic anhydrid with said fibers while a vacuum is maintained, breaking the vacuum when air bubbles substantially cease to evolve from the mixture, and then 70 conducting the acetylating reaction under a pressure at least atmospheric.

Signed at Rochester, New York, this 19th day of Aug., 1927.

HARRY LE B. GRAY.